

## UNITED STATES PATENT OFFICE

2,143,334

## CASEIN PAINT

Wellington Lee Tanner, Panasoffkee, Fla.

No Drawing. Application May 28, 1937,  
Serial No. 145,383

2 Claims. (Cl. 134—50)

My invention relates to paints and processes to compound the same, and more particularly to paints in which the dispersion of casein in an alkaline solution forms the vehicle for the pigments, and my main object is to compound a paint of this nature which is stable and retains its adhesive qualities.

A further object of the invention is to employ an improved formula for compounding paints with a casein content, whereby to render the paint coating or film immune to hydrolyzation and consequent decomposition, and so enable it to retain its firm and integral state.

Another object of the invention is to employ a novel process to compound the paint, whereby to enable a hydro-carbon to be joined as a co-factor with the casein and form a preservative for the resulting product.

In the conventional practice of compounding paints with a casein factor, an aqueous alkaline solution for the dispersion of the casein is considered a good vehicle for carrying the paint pigments. However, paints so compounded have proved unstable whenever exposed to moist air, due to chemical changes occasioned in the casein vehicle by the absorption of moisture. Thus, the casein dispersion becomes completely hydrolyzed in time, and the paint coating or film softens, disintegrates and separates from the surface 30 which it coats.

One method commonly used for fortifying paints prepared with casein is by the admixture of drying oils. While these improve and immunize the product to chemical hydrolysis, they cause poor adhesion of the paint coating to surfaces which are damp; also, the oils impart a glazed or shiny finish to the paint coating which lends glare and harshness to light in contrast with less lustrous finishes, and is therefore less desirable.

So far, no standard casein paint compound meets all requirements, and it has therefore been my intention to develop a paint compound which remains stable and permanent under all atmospheric conditions.

In accordance with the foregoing, my preferred formula for compounding the novel paint is as follows, on a quantitative basis:—

|                                  | Parts |
|----------------------------------|-------|
| 50 Casein, finely ground         | 10    |
| Borax, finely ground             | 2     |
| Pigments, finely ground          | 85    |
| Aluminum stearate, finely ground | 1     |
| Water                            | 50    |
| 55 Toluol                        | 2     |

The above formula is not critical as to the quantities of the ingredients, although experiments have proved that the proportions given result in a superior product. Neither is the formula limited to the specific substances. Thus, any mild alkaline salt may replace the borax. The pigment may be lithopone or the like. The aluminum stearate may be replaced by any other water-insoluble metallic soap of stearic, palmitic or other fatty acids. And a hydrocarbon such as xylol may be substituted for the toluol.

The above ingredients may be compounded by first mixing the powdered ingredients—casein, borax and pigments—into the water in a closed vessel, and then passing the toluol in vaporized form into the vessel, to condense and produce the solvency action. A good paint product is obtained by this method.

Another method of compounding the above ingredients utilizes a closed vessel provided with a strong agitator and jacketed with heating coils. The powdered ingredients are first introduced, and the water added as the agitators operate, until the mass attains a temperature of 80 degrees centigrade or slightly higher. Then, as the stirring continues the hydrocarbon toluol or xylol is introduced in the proper proportion, until the contents reach the finishing stage, forming a product of good quality.

A third method for compounding the ingredients utilizes the water in the form of wet steam. Thus, the dry ingredients are placed, as before, in a closed vessel equipped with strong agitators and jacketed with heating coils; and a condensing coil is provided, to return vapors to the vessel in condensed or liquid form. Now, while the agitators, heating coils and condenser are in action the required amount of the toluol or other hydrocarbon is introduced and followed by the continuous injection of live or wet steam until the vessel contents under agitation have reached the desired volume. A superior paint product is obtained by this method.

The values contributed by the above ingredients to produce the novel paint are of essential importance. Thus, the casein forms a binder and substitute for the usual drying oil vehicle. The borax promotes the dispersion of the casein. The metallic soap functions as a water resistant and commingles with the molecules of the paint pigments to immunize them from hydrolyzation. The water provides the requisite consistency. The toluol is a selective solvent for the metallic stearates and creates a solution which more read-

ily penetrates the compound and envelopes the pigment particles.

It will be evident from the above description that I have improved the manufacture of paints by utilizing the excellent emulsifying property of casein when properly dispersed in a water vehicle. I can thus commingle the hydrocarbon and metallic soap thoroughly with the casein dispersion and produce a paint which has body, adhesive quality, endurance and immunity to hydrolyzation.

I claim:

1. A casein paint composition comprising water as a vehicle, a quantity of pigment in excess by weight of the amount of water, casein dispersed in the water, a small amount of dissolved alkaline agent to maintain dispersion of the casein, the weight of casein being less than the weight of pigment to serve as the paint body and the pigment vehicle in the ultimate coat of paint, a quantity of a water-resistant water-insoluble metallic soap in weight less than the casein, and a

volatile water-immiscible solvent for the said soap, the soap and solvent forming a solution homogeneously dispersed in said vehicle to provide solid soap as a water-proofing agent in the ultimate coat of paint.

2. A casein paint composition comprising water as a vehicle, a quantity of pigment in excess by weight of the amount of water, casein dispersed in the water, a small amount of borax dissolved in the water to maintain dispersion of the casein, the weight of casein being less than the weight of pigment to serve as the paint body and the pigment vehicle in the ultimate coat of paint, a quantity of aluminum stearate in weight less than the casein, and a volatile water-immiscible solvent for the aluminum stearate, the solvent and the aluminum stearate forming a solution homogeneously dispersed in said vehicle to provide solid stearate as a water-proofing agent in the ultimate coat of paint.

WELLINGTON LEE TANNER.

5

10

15

20